

J. T. JONES.  
METALLURGICAL PROCESS.  
APPLICATION FILED DEC. 13, 1917.

1,288,422.

Patented Dec. 17, 1918.



WITNESSES  
*George C. Mayes*

INVENTOR  
**JOHN T. JONES.**

BY *Wm. H. Do.*  
ATTORNEYS

# UNITED STATES PATENT OFFICE.

JOHN TYLER JONES, OF PITTSBURGH, PENNSYLVANIA, ASSIGNOR TO THOMAS J. HOWELLIS, OF PITTSBURGH, PENNSYLVANIA.

## METALLURGICAL PROCESS.

1,288,422.

Specification of Letters Patent. Patented Dec. 17, 1918.

Application filed December 13, 1917. Serial No. 206,994.

To all whom it may concern:

Be it known that I, JOHN TYLER JONES, a citizen of the United States, and a resident of Pittsburgh, in the county of Allegheny and State of Pennsylvania, have invented a new and useful Improvement in Metallurgical Processes, of which the following is a specification.

My invention relates to improvements in metallurgical processes, and it consists in the various steps hereinafter specified.

An object of my invention is to provide a process by means of which metals such as iron and manganese may be economically reduced from their ores to the metallic state.

A further object of my invention is to provide a process in which ores containing iron and manganese may be treated economically, and in which the iron, after it has been reduced to the metallic state, may be easily separated from the manganese, and in which the manganese may subsequently be reduced to the metallic state and separated from the slag.

25 A further object of my invention is to provide a process by means of which iron and manganese when mixed as in an ore, may be reduced to the metallic state, and in which the separation of the iron and the manganese is accomplished by an initial heat treatment which is of high enough temperature to bring the iron in the metallic state, but which is not of sufficient temperature to metallize the manganese, so that the iron 30 may be separated prior to the separation of the manganese, by magnetic means or otherwise.

35 A further object of my invention is to provide a process for treating ores containing iron, manganese and silica, which requires a relatively small amount of coal or other carbonaceous material.

40 Other objects and advantages will appear in the following specification, and the novel features of the invention will be particularly pointed out in the appended claims.

45 My invention is illustrated in the accompanying drawing forming a part of this application, in which, a section of a furnace is shown, this furnace being used in one form of the process.

50 The particular ore which I have in mind in the practice of my process is that found on the Cuyuna range in Minnesota, but the process is equally applicable to ores found

in other regions and of different compositions.

The Cuyuna ore contains the oxids of iron, manganese and silicon in varying proportions, together with small quantities of other elements whose presence, however, does not interfere with the successful carrying out of the process. One part of bituminous coal is finely divided by means of a crusher or any other suitable device, to a fineness ranging from 20 to 100 mesh. Five parts of ore is also crushed to a corresponding fineness and the crushed ore and coal is then intimately mixed.

55 The mixture is placed in a furnace, such as a Siemens regenerative coking oven, and is heated substantially out of the presence of air, to a temperature of substantially 2000° Fahrenheit or to such a temperature as is sufficient to metallize the iron. Care should be taken not to greatly exceed this temperature, because if the temperature approaches 3000°, more of the manganese will be changed to the metal state. By keeping the temperature down, the iron may be recovered in a purer state. On the other hand, it is necessary of course, to have a temperature which metallize substantially all the iron and this, as stated, is approximately 2000° Fahrenheit.

60 The time of this heat treatment varies in accordance with the bulk of material to be treated. For some charges twenty-four hours is sufficient, for others forty-eight, and for others seventy-two, these times conforming to the practice of coking coal. I may state that when the mixture is heated in a crucible, the coking action may be accomplished in a short time, as for instance, in a few minutes.

65 At the end of the coking period, a mixture which is spongy in its nature and semi-plastic when red-hot, is produced, and this is drawn out in a similar manner as coke is drawn from the oven, and cooled by pouring over the mass cold water.

70 The cooled mass is then crushed between rolls and the crushed product is passed through a magnetic separator to take out the iron. The iron occurs as small globules, these globules being of greater or less size but resembling bird-shot so that they are readily separated from the coked product.

75 The pulverized product which remains when the iron is separated, is a silicate of

2  
manganese mixed with particles of carbon. This pulverized mixture is further mixed with lime and put into a furnace adapted to melt the manganese. The particular type of 5 furnace forms no part of the present invention. Any suitable furnace such as an electric furnace which will raise the temperature to substantially that required to melt the manganese might be used. In case there 10 should be an excess of manganese oxid, then an additional amount of carbon in the form of coal may be added with the lime.

15 The melted manganese may be run off from the slag which consists largely of silicate of lime.

20 A modified form of the process consists in adding lime to the mixture of ore and coal before the first heat treatment. To this end, I may take say, twenty (20) parts of ore, 25 four (4) parts of coal, and five (5) parts of lime, by weight, the ore and the coal being pulverized as before stated. The mixture is heated in an oven to substantially 2000° Fahrenheit, substantially out of the presence 30 of air, and the product is a spongy mass consisting of metallic iron in globules, manganese silicate, and silicate of lime, together with particles of coke. This mass is cooled in the manner already described and then is 35 crushed and passed through a magnetic separator. The iron is separated out from the mass and the residue consisting of manganese silicate and silicate of lime, and coke, is passed over a separating table such as a 40 Wilfley table, which separates the manganese from the remaining portion. The separated manganese is then put into an electric furnace and is melted down into the pig.

45 A third form of the process consists in mixing crushed ore and coal in equal parts by weight, heating the same in a coking oven substantially out of the presence of air, and forming a coke-like product consisting of iron in the metallic state but not in the globular state. This iron is in a very 50 finely divided form and is separated by particles of coke. The temperature at which the coking process is carried out is, as in the other forms of the process, substantially 55 2000°, or that temperature which is sufficient to metallize the iron but not the manganese. The product is cooled in the manner already described, and is then put into an open furnace and heated to 2000° or 60 thereabout, air being admitted during the heating process. In the drawing I have shown one form of furnace that might be used. It consists of a vertical chamber 1 open at its top and provided with air openings 2 toward the bottom. Below the air openings are openings 3. The chamber 1 rests on a base 4 which is provided with a trough 5 filled with water 6. The coked mass 7 is fed in at the top of the furnace 65 and the material is continually raked from

the bottom of the furnace through the openings 3 into the trough 5. As the charge descends, additional material is fed in at the top, so that the operation is continuous. In practice it takes about four hours for the 70 charge to pass through the furnace and out into the trough. During the heating process, the iron which was in a finely divided metallic form, is now brought into the nodular form. By keeping the temperature 75 down, that is to say, at point where the iron will be melted but the manganese will not, very little manganese will be found mixed with the iron. The latter may be separated magnetically. The residue containing the 80 manganese, coke and the silica, is heated at a temperature which will melt the manganese, and the latter can be then collected in pig.

85 Each of these forms of the process has certain generic features. In the first place, the material to be operated on is substantially the same. The best results are obtained by finely dividing the ore and the coal in each instance. In each instance, the charge is 90 first coked at a comparatively low temperature, that is to say, at a temperature which is sufficient to metallize the iron but not the other metals, and finally, the iron is separated prior to the separation of the manganese, after which the manganese is melted.

95 I have spoken of the coal and ore as being finely divided. It will be understood that the process is most successfully carried out by finely dividing these materials, but it 100 may be carried out with the materials in lump form, and I therefore consider as falling within the scope of this specification any process which makes use of steps in which the materials are treated in accordance with 105 the foregoing description while in lump form.

110 It will also be noted that I have specified hereafter in the claims hydrocarbon bearing material as a reducing agent. Actual practice shows that the reduction may be accomplished with pure coke. In lieu of a better generic term it will be understood that the term hydrocarbon bearing material 115 includes coke.

11 I claim:

12 1. The herein described metallurgical process which consists in mixing a finely divided ore containing iron and manganese with a finely divided carbonaceous material, heating the mixture substantially out of the presence of air to coke the carbonaceous material and to reduce the iron to the metallic state, separating out the metallic iron, and subsequently reducing the manganese to the 12 metallic state.

13 2. The herein described metallurgical process which consists in mixing a finely divided ore containing iron and manganese with a finely divided carbonaceous material, heat-

ing the mixture substantially out of the presence of air to coke the carbonaceous material and to reduce the iron to the metallic state, separating out the metallic iron magnetically, and subsequently reducing the manganese to the metallic state.

3. The herein described metallurgical process which consists in mixing finely divided ore containing iron and manganese with finely divided coal, coking the mixture at a temperature sufficient to reduce the iron to the metallic state but below a temperature sufficient to reduce the manganese to a metallic state, separating the iron magnetically from the coked mixture, and subsequently heating the residue at an increased temperature to bring the manganese to the metallic state.

4. The herein described metallurgical process which consists in pulverizing an ore containing iron and manganese to substantially twenty to one hundred mesh, pulverizing coal to the same fineness, mixing the pulverized coal with the pulverized ore, heating the mixture substantially out of the presence of air to a temperature of substantially 2000° to coke the coal and to bring the iron into the metallic state, separating the iron from the coked product, and subsequently heating the residue at an increased temperature to bring the manganese into the metallic state.

5. The herein described metallurgical process which consists in pulverizing an ore containing iron and manganese to substantially twenty to one hundred mesh, pulverizing coal to the same fineness, mixing the pulverized coal with the pulverized ore, heating the mixture substantially out of the presence of air to a temperature of substantially 2000° to coke the coal and to bring the iron into the metallic state, separating the iron from the coked product, and subsequently heating the residue to substantially 3000° Fahrenheit, in the presence of air to bring the manganese into the metallic state.

6. The herein described metallurgical process which consists in heating a finely divided ore containing iron and manganese with finely divided coal substantially out of the presence of air at a temperature which will coke the coal and will bring the iron to the metallic state, and which will also substantially prevent the bringing of the manganese into the metallic state, adding lime

to the residue, heating the residue in the presence of air to a temperature sufficient to melt the manganese and to form silicate of lime.

7. The herein described metallurgical process which consists in pulverizing an ore containing iron, manganese and silica, mixing the pulverized ore with pulverized coal, heating the mixture substantially out of the presence of air at a temperature sufficient to coke the coal and to bring the iron into the metallic state, but which will not melt the manganese, crushing the coked mixture, separating out the iron magnetically, adding lime to the crushed residue, heating the residue at a temperature sufficient to melt the manganese and to form silicate of lime.

8. The herein described metallurgical process which consists in mixing pulverized ore containing iron, manganese, and silica, with pulverized coal in the proportions of one part of coal to five parts of ore, heating the mixture substantially out of the presence of air at a temperature sufficient to melt the iron and to coke the coal but not sufficient to melt the manganese, cooling and crushing the coked product, separating out the iron magnetically, adding lime to the crushed residue, heating the crushed residue with the admixture of lime in the presence of air to a temperature sufficient to bring the manganese into the molten state and to form silicate of lime, and separating the metal from the silicate.

9. The herein described metallurgical process which consists in mixing finely divided ore containing iron and manganese with finely divided coal, coking the mixture at a temperature sufficient to reduce the iron to the metallic state but below a temperature sufficient to reduce the manganese to a metallic state, separating the iron from the coked mixture, and subsequently heating the residue at an increased temperature to bring the manganese to the metallic state.

10. The herein described metallurgical process which consists in mixing ore containing iron and manganese with a carbonaceous material, heating the mixture substantially out of the presence of air to coke the carbonaceous material and to reduce the iron to the metallic state, separating out the metallic iron and subsequently reducing the manganese to the metallic state.

JOHN TYLER JONES.